

## UNITED STATES PATENT OFFICE

1,971,036

## FLOOR COVERING AND METHOD

James E. Graham, Needham, and Edwin M. Lines,  
Dedham, Mass., assignors to Bird & Son, Inc.,  
East Walpole, Mass., a corporation of Massachusetts

No Drawing. Application November 6, 1933,  
Serial No. 696,834

14 Claims. (Cl. 91—67.9)

This invention relates to a floor covering of the hard-surfaced flexible type and method of making the same, and has particularly to do with a resilient floor covering which has advantages and properties not found in other hard-surfaced floor coverings such as felt base rugs and linoleum.

The invention provides a hard-surfaced flexible floor covering that is not only attractive in its decoration but is extremely tough and durable, relatively non-saponifying and non-water absorbent, as well as resistant to fats, oils, grease, etc., and which can nevertheless be manufactured economically and be ready for sale and use in a minimum of time, in fact within a period of a day or two. In addition to these properties the product of this invention due to its novel composition and structure has a wear resistance not found in printed felt base floor coverings since the wearing layer is formed from a plastic and relatively thick and the decoration of the floor covering of this invention as distinguished from said felt base floor coverings is not simply upon the surface but, on the contrary, extends well into and impregnates the said wearing layer of our novel product.

Felt base floor coverings are solely dependent for their wear-resistant qualities upon a few coats of pigmented paint including a printed design, sometimes supplemented by an additional coat or coatings of transparent varnish, lacquer, or the like. Printed linoleum is in the same category and the decorative appearance is soon lost due to ordinary usage. In the better grades of linoleum the color or pigment is added to the linoleum mixture being either a plain color, variegated or mottled, or, as in inlaid linoleum, made from different colored mixtures applied in separate areas. With such plastic material, however, it has not been possible to obtain delicate designs and effects because of the difficulty in working the plastic mixtures in fine lines, nor has it been practical or possible commercially to color a substantial thickness of the wearing layer of linoleum by means of after-applied coloring material or dyes because the linoleum mixtures, due to the waterproof and water-resistant character of the linoxyn binder will not permit the ingress of such inks or dyes. The floor covering of this invention embodies a wearing layer of substantial thickness made from a novel plastic composition (as hereinafter more fully described) which is frictioned in layer form in situ as it is applied in substantial thickness to a base or backing of woven or felted sheet material.

55 The plastic composition as hereinafter more fully

described comprises in its preferred form a mixture of what is essentially non-fibrous wood powder, that is, wood so finely divided as to, as a practical matter, eliminate its fibrous characteristics, and binders, at least one of said binders including as the essential constituent thereof, a cellulose ester,—nitro-cellulose being preferred for this purpose because of its ability to produce a tough elastic layer and to cement or bond the wood powder, because of its high resistance to wear, and because it makes an excellent bond with any one of various backing or reinforcing materials. Nitro-cellulose alone has, however, certain characteristics which are objectionable for the purpose of a binder, among which may be mentioned particularly the fact that it is brittle, difficult to work, and also, it does not adhere well to a backing or reinforcing material, for example, a bitumen impregnated felt base, coated or uncoated. One or more plasticizers such as tricresyl phosphate or ester gum, hereinafter mentioned, must be incorporated therewith as hereinafter more fully described. To find a satisfactory solution for the problems presented by these conditions has involved a long series of experiments and testing of products.

Though it would seem that such a plastic, including a waterproof binder as described, would neither be permeable nor receptive to a coloring dye because of the waterproof character of the cellulose ester binder constituent as described, we have found that with the combination of wood powder and binder as herein described, the plastic mixture has sufficient tenacity so that it can be frictioned upon and adhere to a backing, and still be sufficiently permeable to dyes as to permit a coloring extending through or substantially through the vertical depth or thickness of the wearing layer by simply printing or otherwise applying such dyes upon the exposed surface of the plastic composition after having been frictioned to the base as described.

Following the coloring of the plastic mixture and the drying off of the dye solvent, there is applied and incorporated into the wearing layer, as an essential constituent thereof, an additional or supplementary binder which serves to fill up the pores in the dried plastic mixture and thus render the resultant product impermeable to liquids and still more firm and wear-resistant.

As an example of the manufacture of floor covering in accordance with this invention we give the following as the present preferred practice thereof. A suitable flexible backing or base is first prepared which preferably is an asphalt-

saturated felt, but any suitable woven, felted or sheeted material may be employed. To one surface of the base material is applied an under-coat or filler to prevent staining by the asphalt 5 of the after-applied wearing layer. To the base there is then applied a plastic mixture as follows (all parts being by weight):

30-50 parts nitro cellulose (average viscosity 15-20 sec.)

10 45-75 parts tricresyl phosphate

20-40 parts ester gum solution (2% gum and  $\frac{1}{3}$  solvent)

15 40-60 parts mineral pigment (usually white or neutral in color, though, if desired, the plastic composition may be colored as required by colored mineral pigment)

20 250-350 parts wood powder (substantially all passing a 60 mesh screen, at least  $\frac{1}{2}$  passing a 100 mesh screen, and a substantial portion passing 20 a 200 mesh screen)

100-150 parts nitro-cellulose solvent (butyl acetate, alcohol, etc.)

This mixture is, by suitably driven rolls, frictioned in situ in layer form to the base to the 25 thickness desired (say .015"-.030") and the product then dried from two to eight hours at 100° F. As the result of this drying the solvent passes off leaving the wood powder held together by the primary binder, thus providing a very open 30 and porous structure which will take up about 75% of its own weight of a liquid. If colored plastic material is employed, the layer may include a single color or several colors, the latter giving to the frictioned layer before printing a 35 marbleized or Jaspé appearance. This may be accomplished by depositing the differently colored plastics in the frictioning calendar.

Following the drying of the intermediate product it is ready for the coloring or decorating 40 step which may be done by printing on a flat bed print machine with the same type of print blocks as are commercially used for printing felt base rugs, but any method of applying color, rotary or flat bed, may be used. In the commercial practice of this invention for coloring 45 the wearing layer, we preferably employ water-soluble dyes (together with a very small amount of a thickening agent such as gum tragacanth) though oil and spirit soluble dyes are usable. The liquid color is ordinarily applied in an amount 50 equal to about 60% of the dry weight of the wearing layer in its porous and liquid-permeable condition. The colored product is then dried, say for a period of from two to four hours in a moderately heated oven, as a result of which, substantially 55 all of the liquid carrier of the dye is evaporated.

The succeeding operation is that of filling up 60 the voids or pores in the colored plastic mixture which still presents an open structure. This is an essential feature of the process and includes the application to the permeable wearing layer of a substantial amount of a binder material or materials, say in an amount approximately 65 one half of the weight of the said colored and dried plastic mixture, of a liquid material adapted to set or harden, for example, drying oil, wax or wax-like materials, resin, lacquer, or the like, or a mixture of two or more of them. In this manner, the pores or voids in the previously applied plastic mixture in effect become 70 saturated throughout its thickness by this after-applied binder and the result is a very marked increase in durability and strength as well as 75 a greatly improved finish. In practice, drying

oils such as linseed and Chinawood have been found satisfactory and there is ordinarily incorporated therewith a small amount of resin in order that the finished product may present a firmer and harder wear-resistant surface. It 80 is also contemplated that the dye (with or without a solvent) may be first mixed with the additional binder and applied to the partially completed wearing layer by the application thereto of the colored binder.

If desired, in order to provide a glossy finish, a top layer or surface coating of varnish or lacquer may be applied, though it is not necessary, for the additional or supplementary binder, if applied in sufficient quantity, completely fills the pores so as to present a water-impermeable 85 surface and one exhibiting an attractive finish.

In the typical preferred product, the completed wearing layer includes 40-50% wood powder, pigment, if desired (as mentioned in the foregoing example), 10-20% initial binder, 1-3% of color, and 30-40% of the after-applied 90 supplementary or filler-binder, this table of constituents being made without regard to the presence or absence of a final finishing coat of transparent varnish or the like, which, if used, may be present in an amount approximately equal to the initial binder material.

Having described our invention, what we wish to claim and secure by Letters Patent is:

1. A hard-surfaced flexible floor covering comprising a base with a wearing layer of substantial thickness formed from a plastic material adhesively united thereto, said wearing layer consisting essentially of substantially non-fibrous, finely powdered wood, a relatively small amount of binder material providing a porous body structure colored through at least a major portion of its vertical depth, to present a design therein and with the pores thereof filled with a hardened 110 binder material in a quantity in excess of said first mentioned binder material.

2. A hard-surfaced flexible floor covering comprising a base with a wearing layer of substantial thickness formed from a plastic material frictioned thereto, said wearing layer consisting essentially of substantially non-fibrous, finely powdered wood, a relatively small amount of binder material providing a porous body structure colored through at least a major portion of its vertical depth, to present a design therein and with the pores thereof filled with a hardened binder 120 material in a quantity in excess of said first mentioned binder material.

3. A hard-surfaced flexible floor covering comprising a base with a wearing layer of substantial thickness formed from a plastic material adhesively united thereto, said wearing layer consisting essentially of substantially non-fibrous, finely powdered wood, a relatively small amount of 135 waterproof binder material providing a porous body structure colored to present a design therein with the said design extending substantially through the vertical depth of said layer and with the pores thereof filled with a hardened binder material.

4. A hard-surfaced flexible floor covering comprising a base with a wearing layer of substantial thickness formed from a plastic material frictioned thereto, said wearing layer consisting essentially of substantially non-fibrous, finely powdered wood, a relatively small amount of binder material providing a porous body structure printed to present a colored design therein, extending through at least a major portion of the vertical 145 material.

- depth thereof, and with the pores thereof filled with a hardened binder material in a quantity in excess of said first mentioned binder material.
5. A hard-surfaced flexible floor covering comprising a base with a wearing layer of substantial thickness formed from a plastic material adhesively united thereto, said wearing layer consisting essentially of substantially non-fibrous, finely powdered wood, a relatively small amount of cellulose ester binder material providing a porous body structure colored to present a design therein, extending through at least a major portion of the vertical depth thereof, and at the exposed surface thereof and with the pores thereof filled with a hardened waterproof binder material in addition to said first mentioned binder material.
6. A hard-surfaced flexible floor covering comprising a base with a wearing layer of substantial thickness formed from a plastic material adhesively united thereto, said wearing layer consisting essentially of substantially non-fibrous, finely powdered wood, a relatively small amount of cellulose ester binder material providing a porous body structure colored substantially throughout its vertical depth to present a design therein with a hardened binder material in a quantity substantially in excess of said first mentioned binder material.
7. A hard-surfaced flexible floor covering comprising a base with a wearing layer of substantial thickness formed from a plastic material adhesively united thereto, said wearing layer consisting essentially of substantially non-fibrous, finely powdered wood, a relatively small amount of cellulose ester binder material providing a porous body structure colored with a dye to present a design therein, extending through at least a major portion of the vertical depth thereof, and with the pores thereof filled with a linoxyn binder material in a quantity substantially in excess of said first mentioned binder material.
8. The method of making a hard-surfaced flexible floor covering which consists in applying to a flexible base a wearing layer of substantial thickness of plastic material and adhesively uniting the same thereto, said plastic material consisting essentially of substantially non-fibrous, finely powdered wood and a relatively small amount of binder material, drying the said intermediate product thus formed, coloring the wearing layer of said product with coloring material with the said coloring material extending through at least a major portion of the vertical depth of said wearing layer, and filling the pores of said wearing layer with additional hardening binder material.
9. The method of making a hard-surfaced flexible floor covering which consists in frictioning to a flexible base a wearing layer of substantial thickness of plastic material and adhesively uniting the same thereto, said plastic material consisting essentially of substantially non-fibrous, finely powdered wood and a relatively small amount of binder material, drying the said intermediate product thus formed, coloring the wearing layer of the same to provide design therein with the said design extending through at least a major portion of the vertical depth of said wearing layer, and filling the pores of said wearing layer with additional hardening binder material.
10. The method of making a hard-surfaced flexible floor covering which consists in friction-
- ing to a flexible base a wearing layer of substantial thickness of plastic material and adhesively uniting the same thereto, said plastic material consisting essentially of substantially non-fibrous, finely powdered wood and a relatively small amount of a binder material, drying the said intermediate product thus formed, coloring the wearing layer of the same by printing to provide a design therein with the said design extending substantially through the vertical depth of said wearing layer, and filling the pores of said wearing layer with additional hardening binder material.
11. The method of making a hard-surfaced flexible floor covering which consists in applying to a flexible base a wearing layer of substantial thickness of plastic material and adhesively uniting the same thereto, said plastic material consisting essentially of substantially non-fibrous, finely powdered wood and a relatively small amount of cellulose ester binder material, drying the said intermediate product thus formed, coloring the wearing layer of the same by printing a design thereon to provide design therein with the said printed design extending through at least a major portion of the vertical depth of said wearing layer, and filling the pores of said wearing layer with additional hardening binder material.
12. The method of making a hard-surfaced flexible floor covering which consists in frictioning to a flexible base a wearing layer of substantial thickness of plastic material and thereby adhesively uniting the same thereto, said plastic material consisting essentially of substantially non-fibrous, finely powdered wood and a relatively small amount of cellulose ester binder material, drying the said intermediate product thus formed, and then applying thereto coloring and additional binding material to fill the pores thereof, with the coloring extending through at least a major portion of the vertical depth of said wearing layer.
13. The method of making a hard-surfaced flexible floor covering which consists in frictioning to a flexible base a wearing layer of substantial thickness of plastic material and thereby adhesively uniting the same thereto, said plastic material consisting essentially of substantially non-fibrous, finely powdered wood and a relatively small amount of a binder material, drying the said intermediate product thus formed, and then applying thereto coloring and additional binding material to fill the pores thereof, with the coloring extending through at least a major portion of the vertical depth of said wearing layer.
14. The method of making a hard-surfaced flexible floor covering which consists in frictioning to a flexible base a wearing layer of substantial thickness of plastic material and thereby adhesively uniting the same thereto, said plastic material consisting essentially of substantially non-fibrous, finely powdered wood and a relatively small amount of a binder material, drying the said intermediate product thus formed, and then applying thereto coloring and additional binder material in excess of the amount of said first mentioned binder material to fill the pores thereof, with the coloring extending through at least a major portion of the vertical depth of said wearing layer.

JAMES E. GRAHAM.  
EDWIN M. LINES.